

Oct. 21, 1958

R. EASTON

2,856,658

METHOD OF CONTINUOUS CASTING

Filed Aug. 13, 1956



INVENTOR.  
RUFUS EASTON.

BY  
Ralph B. Crick.  
his ATTORNEY

# United States Patent Office

2,856,658

Patented Oct. 21, 1958

1

2,856,658

## METHOD OF CONTINUOUS CASTING

Rufus Easton, Pittsburgh, Pa., assignor to Koppers Company, Inc., a corporation of Delaware

Application August 13, 1956, Serial No. 603,613

2 Claims. (Cl. 22—200.1)

This invention relates to the continuous casting of molten metals and more particularly to a method of continuously casting molten metal in a casting run so as to avoid metal spill-over at the end of the run.

In the continuous casting of molten metals, and particularly in the casting of molten steel, it has been found necessary to stop the downward motion of the solidifying casting after the flow of the metal from the tundish nozzle has stopped until the solidification of the metal has been completed. During this period, there frequently occurs a bending or bowing of the solidifying shell inwardly toward the longitudinal axis of the casting. When this bending takes place, a spill-over of the molten metal core over the shell results. The spill-over runs down between the mold and the shell wall and past the bottom of the mold, with resulting damage to the spray and roller system.

Experts in the art believe that the inwardly bending motion of the shell probably is due to the reheating of the casting near the bottom of the mold along the outer portion of the shell. This reheating has been explained to be a result of the withdrawal of the shell from contact with the mold as the general cooling proceeds. Once the withdrawal takes place, the heat transfer from the casting to the mold wall ceases and the outer portion of the shell, which had been cooled down, reheat, expanding as it does so. Since there is no appreciable change in temperature in the inner portion of the shell and therefore no appreciable change in length, the expansion of the outer portion of the shell results in an inward bowing or bending of the shell away from the mold wall. When this occurs, the abovementioned undesirable spill-over of the molten metal core surrounded by the solidifying shell results at the end of the run. It then is necessary to repair the resulting damage caused by the spill-over before casting operations can commence again.

The present invention avoids the abovementioned disadvantages by providing an economical, efficient, and straightforward method which prevents spill-over at the end of the run. Various other features of the present invention will become obvious to one skilled in the art upon reading the disclosure set forth hereinafter. More particularly, the present invention provides a method of continuously casting molten metal comprising freely passing a supply of molten metal from a point spaced above an open-ended mold through such open-ended mold in a casting run, cooling the metal as it passes through the mold during the run to form a solidifying shell about the molten metal core, and supporting the solidifying shell against the mold wall at the end of the run to prevent spill-over.

It is to be understood that various changes can be made by one skilled in the art in the several steps of the method disclosed herein without departing from the scope or spirit of this invention.

2

Referring to the drawing, a schematic view is disclosed of a mold at the end of a casting run, which run included the practice of the method of the present invention.

More particularly, an open-ended mold 2 is disclosed, the mold having an inner wall 3. A plurality of spaced support and guide rollers 4 are positioned below the mold. It is to be understood that the practice of the present inventive method is not to be limited to the specific mold structure disclosed, but that various other mold and roller arrangements can be used in carrying out the several steps of the invention.

A supply of molten metal has been furnished to mold 2 from a tundish nozzle (not shown) in a typical casting run and, as can be seen in the drawing, the casting in the mold, broadly designated by reference numeral 6, has developed a solidifying shell 7 which surrounds molten metal core 8. Since, as above discussed, there is a tendency for the solidifying shell in the mold 2 to bend and buckle inwardly to bring about undesirable molten metal spill-over, a supporting unit 9 has been inserted into the molten metal core at the end of the run.

In the advantageous embodiment of the invention disclosed, the supporting unit 9 is in the form of a C-shaped piece of bent round iron bar, the legs 11 of the bar being positioned to hold the sides of the shell 7 against the wall 3 of mold 2. In this connection, it is to be understood that the particular shape of supporting unit 9 can vary in accordance with the type of mold used and results desired. It is to be further understood that the supporting unit can be made from any number of well known types of materials, and although advantageously a C-shaped iron member has been found satisfactory, it also is possible to use effectively refractory materials of various shapes to accomplish the support.

It is to be noted that the supporting unit can be inserted into the mold manually by means of a pair of gripping tongs. Further, it is to be noted that the unit should be inserted promptly at the end of the run, advantageously within 20-30 seconds after the molten metal has ceased to flow from the tundish. With the supporting unit properly inserted, the metal continues to solidify, but the supporting structure resists any inward bending of the solidifying shell 7, thus avoiding any spill-over of the molten metal core 8 surrounded by the shell.

The invention claimed is:

1. A method of continuously casting molten steel comprising passing a supply of molten steel through an open-ended mold in a casting run, cooling said steel as it passes through the mold during the run to form a solidifying shell about a molten metal core, and promptly inserting into the molten metal core at the end of the run a C-shaped support bar to maintain the solidifying shell of the casting against said mold to prevent spill-over.

2. In a method for continuously casting a billet of solid cross-section comprising passing a stream of molten metal through an open-ended mold, cooling said molten metal externally as it passes through said mold to form a solidifying external shell about a gradually solidifying molten metal core, terminating the flow of said stream of molten metal through said mold, and inserting a member into said gradually solidifying molten metal core to maintain the solidifying shell of the casting spread outwardly against said mold to prevent spill over.

References Cited in the file of this patent

UNITED STATES PATENTS

|           |        |                |
|-----------|--------|----------------|
| 2,048,734 | Eldred | July 28, 1936  |
| 2,130,202 | Tama   | Sept. 13, 1938 |
| 2,277,375 | Tama   | Mar. 24, 1942  |